

## UNITED STATES PATENT OFFICE

2,108,243

## PHOTOGRAPHIC DEVELOPER

Bruno Wendt, Dessau, Germany, assignor to Agfa  
Ansco Corporation, Binghamton, N. Y., a cor-  
poration of New York

No Drawing. Application July 16, 1936, Serial  
No. 90,919. In Germany July 23, 1935

5 Claims. (Cl. 95—88)

My present invention relates to a photographic developer and more particularly to a developer for development in colors.

One of its objects is to provide an improved developer. Another object is to provide an improved developer for development in colors. Further objects will be seen from the detailed specification following hereafter.

Para-phenylenediamine is used as a fine-grain developer and derivatives of para-phenylenediamine have been proposed as developers. The latter compounds, however, have not been introduced into photographic practice because their speed in developing is relatively low.

This invention relates to a process of photographic development in which N-hydroxyalkylated para-phenylenediamines are used as developers. Examples of suitable compounds are unsymmetrical dihydroxydiethyl-para-phenylenediamine, methyl-hydroxyethyl-, ethyl-hydroxyethyl-, butyl-hydroxyethyl-para-phenylenediamine, as well as the corresponding toluidines. Also  $\beta$ - $\gamma$ -dihydroxy-propyl-para-phenylenediamines, such as the diamine itself and its alkyl derivatives. These compounds are obtainable by known methods from the corresponding aniline derivatives, the latter being converted into the nitroso-derivative and the nitroso-group being then reduced; or by coupling the hydroxy-alkyl-aniline derivative with an azo-component, for instance diazotized sulfanilic acid, to make an azo-dyestuff which is then reduced in the usual manner.

The unsymmetrical dihydroxy-diethyl-para-phenylenediamine may be made from dihydroxy-diethyl-aniline by converting the latter into its nitroso-derivative and reducing the nitroso-group. Developers made with this compound develop about three times more quickly than that made from non-substituted para-phenylenediamine and also yield very fine-grain negatives.

The developers have particularly good solubility, which is to be attributed to the hydroxyalkyl-group. Furthermore, the developers are particularly useful for development in color, since they have the advantage over the normal alkyl-derivatives that they yield purer and brighter colors. For the purpose of development in color there may be added to the developer besides the developing substance, substances which have a tendency to produce dyestuffs during the development by oxidation of the developer, for instance, a derivative of acylacetic acid ester for the production of a yellow color, pyrazolones for the production of a red color, and a derivative of 1-hydroxy-

naphthalene-2-carboxylic acid for the production of a blue color.

The following examples illustrate the invention:

## Example 1

5 A developer consisting of:

10.9 grams of unsymmetrical N,N-di-(hydroxyethyl)-para-phenylenediamine

60 grams of anhydrous sodium sulfite

1000 cc. of water

yields a  $\gamma$ -value of 0.6 after 25 minutes in a given emulsion. On the other hand, a developer consisting of:

15 6 grams of para-phenylenediamine

60 grams of anhydrous sodium sulfite

1000 cc. of water

and containing the same number of molecules of the developing substance, yields in the same given emulsion a  $\gamma$ -value of 0.6 only after 75 minutes.

## Example 2

A developer consisting of:

25 10 grams of 2-amino-5-(N-hydroxyethyl-N-butyl)-amino-toluene-dihydrochloride

10 grams of dibromo-ortho-cresol

3.5 grams of caustic soda

1000 cc. of water

yields a green picture, whereas the known developers having dibromocresol as a constituent yield only a blue-green color.

## Example 3

35 9.0 grams of N-ethyl-N-hydroxyethyl-p-phenylene-diamine

60.0 grams of anhydrous sodium sulfite

0.5 gram of potassium bromide

1000 cc. of water

## Example 4

First solution:

1.0 gram of N,N-di-(hydroxyethyl)-p-phenylene-diamine

100 cc. of water.

Second solution:

0.9 gram of phenyl-methyl-pyrazolone

4.0 grams of anhydrous sodium carbonate

100 cc. of water.

## Example 5

First solution:

55

1.0 gram of N,N-di-(hydroxyethyl)-p-phenylenediamine  
100 cc. of water.

5 Second solution:

0.9 gram of o-phenyl-phenol  
0.4 gram of caustic soda  
100 cc. of water.

10 In Examples 4 and 5 the two solutions are mixed before use.

What I claim is:

1. A photographic developer comprising an N-hydroxyalkylated p-phenylenediamine.
2. A photographic developer comprising an N-

hydroxyalkylated p-phenylenediamine and a compound capable of forming a dye with the oxidation products of the developer.

3. A photographic developer comprising unsymmetrical N,N-di-(hydroxyethyl)-p-phenylenediamine. 5

4. A photographic developer comprising N-ethyl-N-hydroxyethyl-p-phenylenediamine, anhydrous sodium sulfite, potassium bromide and water. 10

5. A photographic developer comprising N,N-di-(hydroxyethyl)-p-phenylenediamine, o-phenyl-phenol, caustic soda and water.

BRUNO WENDT.